

Dec. 21, 1948.

G. W. W. STEVENS

2,457,005

PHOTOGRAPHIC PROCESS

Filed Aug. 1, 1947

2 Sheets-Sheet 1



GUY WILLIAM WILLIS STEVENS  
INVENTOR

H. M. Perrins  
BY Daniel J. Mayne  
ATTORNEYS

Dec. 21, 1948.

G. W. W. STEVENS  
PHOTOGRAPHIC PROCESS

2,457,005

Filed Aug. 1, 1947

2 Sheets-Sheet 2



GUY WILLIAM WILLIS STEVENS  
INVENTOR

By *H. M. Perrins*  
*Daniel J. Mayne*  
ATTORNEYS

## UNITED STATES PATENT OFFICE

2,457,005

## PHOTOGRAPHIC PROCESS

Guy William Willis Stevens, Harrow, Wealdstone, England, assignor to Eastman Kodak Company, Rochester, N. Y., a corporation of New Jersey

Application August 1, 1947, Serial No. 765,635  
In Great Britain January 31, 1945

6 Claims. (Cl. 95—5)

1

This invention relates to photographic processes and to material therefor.

In the copending application of Edward B. Knott and Guy W. W. Stevens, Serial Number 765,636, filed August 1, 1947, there is described a method for selectively producing images in a photographic material comprising an inseparable combination of silver salt emulsions on a single support which comprises employing two emulsions of different types (type I—an emulsion which forms the latent image mostly inside the silver salt grains; and type II—an emulsion which forms surface latent image on the silver salt grains), selectively exposing (simultaneously or consecutively) both emulsions to form latent images therein, and then differentially developing the latent images so formed.

In the copending application of Edward B. Knott and Guy W. W. Stevens, Serial Number 765,632, filed August 1, 1947, there is described a method for producing a reversed photographic image, which comprises exposing to an object or image a sensitive layer comprising a silver salt emulsion of the aforesaid type I (an emulsion which forms the latent image mostly inside the silver salt grains), then, without developing the latent image so formed to a visible image, treating the emulsion to render it capable of forming surface latent image, and then subjecting it directly (i. e. not through a negative or positive image) to an exposure of sufficient intensity and time to cause a reversed image to develop upon treating the directly exposed emulsion in a developer which will develop surface latent images, but not develop or develop only slightly the first-formed internal latent image.

I have now found that this forms the subject of the present invention that very useful results can be obtained, if in the inseparable combination of silver salt emulsions described in the said copending application Serial Number 765,636, the type I emulsion (an emulsion which forms the latent image mostly inside the silver salt grains) is processed to give a reversed image according to the method described in said copending application Serial Number 765,632, and the type II emulsion (an emulsion which forms surface latent image on the silver salt grains) is processed to give an ordinary image. In a modification of this invention, the type II emulsion is processed by known reversal technique and the type I emulsion is processed to give an ordinary image.

In a preferred form of the invention, the emulsions have different spectral sensitivities and therefore they can be selectively exposed to form

2

the said latent images therein by different coloured lights; such exposures can, of course, with advantage be made simultaneously but this is not essential.

5. If desired a filter layer may be interposed between the two emulsion layers to facilitate the selective exposure thereof. For instance, if a yellow filter layer is interposed, the emulsions can be exposed from opposite sides by means of 10. blue light; this method is useful when printing from two different black and white colour separation records. In many cases it is better to use an interposed filter layer and at the same time use emulsions of different colour sensitivities. For example if a yellow filter layer is used and the one emulsion is dye sensitised to red then on exposing the material (from the side remote from such red sensitive emulsion) to blue and red images simultaneously, the blue 20 image will be recorded in the nearest emulsion and the red image in the other emulsion.

In either form of the present invention there is obtained in one of the two emulsions, a reversed image and in the other of the two emulsions an ordinary (i. e. non-reversed) image.

25. In the above described form of the invention where the image in the type I emulsion is processed to give a reversed image according to the method described in application No. 765,632 and the type II emulsion is processed to give an ordinary image, then if desired, after both images have been developed they may both be reversed by known reversal technique.

30. The method of the present invention is very useful when applied to the production of colour corrected colour photographs, that is to say, where the so-called masking method of colour correction is employed. In such masking methods as applied to reproduction of a multi-coloured object or image, one colour separation record in the form of a negative is printed through a positive transparency of another colour separation record; such positive is of lower overall contrast than the negative, and is 35. known as a mask. The function and method of using such a mask is well known. It has previously been suggested to make the negative and its mask in register on a single support using in superimposition an ordinary emulsion in which 40. the negative is formed and a special emulsion in which the positive is formed as a reversed image on direct development; such direct positive was developed as the result of a positive latent image being first formed by polarization.

45. In the method of the present invention, how-

ever negative latent images are first produced by the initial exposure of both emulsions which means that the effective sensitivities of both emulsions can be very much higher, thus permitting convenient exposures to be made in a camera.

The method of the present invention for masking operations has various advantages over the prior proposals, for instance, it allows of more highly sensitive emulsions being used, and does not involve any difficult treatments such as controlled penetration for selectively processing the superimposed or mixed emulsions.

The following is an illustration of how the present invention is applied to such masking technique. On a glass support, there is first coated an emulsion, for instance a gelatino-silver-chloride emulsion of type II (a gelatino-silver-chloride emulsion which forms surface latent image on the silver halide grains) which is dye-sensitized to the red; and over this emulsion and in direct contact therewith is coated a gelatino-silver-halide emulsion of type I (a gelatino-silver-halide emulsion which forms the latent image mostly inside the silver halide grains) which is not dye-sensitized, either to red or to green. The sensitive material so obtained is then exposed to a multi-coloured object or image through either a red and blue filter successively or through a single filter transmitting both red and blue. The type I emulsion is made to have a sufficiently high speed to insure that the amount of blue light necessary for its correct exposure, is too small to have any practical effect on the type II emulsion. Hence, the red exposure affects only the type II emulsion and the blue exposure only the type I emulsion. The exposed material is then immersed in a "surface" developer (a developer which develops substantially only surface latent image) and given a uniform blue-light exposure just sufficient to form in the type I emulsion a reversed latent image, but insufficient to have any practical effect on the type II emulsion. The material is held in this developer until the negative image (i. e. the red record) is satisfactorily developed in the type II emulsion and during this time a positive image (i. e. the blue record) develops in the type I emulsion.

The said uniform exposure should be made from the side remote from the type II emulsion, so that it is not influenced by the negative image developing up in the type II emulsion. Some convenient control of contrast of the positive image can be obtained by giving the uniform exposure at a suitable time after immersion of the material in the surface developer; for instance, if such exposure is given when the said negative image is almost wholly developed, quite a low contrast will be obtained in the said positive image by the time the negative image is wholly developed.

In the processing technique just described, there is obtained a negative image in the type II emulsion and a positive in the type I emulsion. An advantage given by the present invention is that instead of processing such an exposed material in that way, it can be processed to give a positive image in the type II emulsion and a negative image in the type I emulsion. For instance, this can be done by omitting to give the material a uniform exposure when developing the first-formed negative latent image in the type II emulsion, and then, after such negative image is developed (there being no development so far of the type I emulsion), dissolve out all the silver of such image with a bath which does not destroy

the red-sensitivity of the type II emulsion, nor destroys the internal image of the type I emulsion. Next give a uniform red light exposure to the material preferably from the side remote from the type I emulsion, and then immerse the material in an "internal" developer (a developer which develops latent image inside the silver salt grains), whereupon a positive image develops in the type II emulsion and a negative image in the type I emulsion. Where the type I emulsion is more stable to fogging developers than is the type II emulsion, as is especially the case when the type II emulsion is a silver chloride emulsion, the following alternative procedure can be adopted. The said uniform red light exposure is omitted and then only the type I emulsion develops in the internal developer; after this step, the material is treated with a fogging developer which will rapidly develop the residue of the type II emulsion without effecting the silver halide remaining in the type I emulsion.

Still another way of processing the material consists in treating it (after the exposure to the multi-coloured object or image) in a "surface" developer so as to develop only the type II emulsion, and then removing the silver so produced. Next treat with an "internal" developer so as to develop a negative image in the type I emulsion. Then treat with a solution which restores the type I emulsion to its original condition, in which it cannot form surface latent image (the first treatment in a surface developer having previously made it capable of forming surface latent image), and give a uniform exposure (which may be blue) so as to fog the remaining silver halide of the type II emulsion and develop this only in a surface developer.

It will be seen that in some of the cases illustrated above, the same material and same image exposure (i. e. the first exposure) can be used to give at will either a positive of the one colour record and a negative of the other or vice versa.

Although the above described processing procedures are given with reference to the particular material given above, it is to be understood that analogous procedures can be applied to material with colour sensitivities different from those given above. Thus in some cases it may be convenient to employ a type I emulsion having a relatively low speed in the blue to blue-green portion of the spectrum but dye sensitised to red and a type II emulsion having a relatively high speed in the blue to blue-green portion of the spectrum. Alternatively, if instead of recording red and blue respectively in the two emulsions, it is desired to record green and blue respectively, then instead of the type II emulsion being sensitised in well known manner to red and not green, as indicated above, it can be sensitised to green and not to red; the subsequent exposure to a multi-coloured object will then, of course, be to green and blue light.

Another use to which the method of the present invention can be put is in the selective recording of coloured parts of a multi-coloured record. For instance, if a map, or other drawing consists of say red lines, blue lines, magenta lines and black lines, then a record of only the blue lines (for example) can be easily obtained. One way in which this can be done will now be given by way of illustration.

#### EXAMPLE

A support, such as a glass plate was coated first with a contrasty, low blue speed gelatino-sil-

ver-chloride emulsion (type II) sensitized to the red with 0.15 g. of 3,3'-dimethyl-9-ethyl-4,5,4',5'-dibenzothiacarbocyanine iodide, the carbocyanine dye being added to an amount of the emulsion containing 165 g. of silver chloride, to give an emulsion layer containing 0.4 g. of silver per square foot. This emulsion layer was then coated with a type I gelatino-silver bromiodide emulsion of high speed (relative to the type II emulsion) in the blue-to-blue-green portion of the spectrum and having little or no green or red sensitivity to give an emulsion layer containing 0.9 g. of silver per square foot superimposed on the first emulsion layer.

The resulting sensitive photographic plate was then exposed to a drawing, such as a map, composed of blue, red, green and black lines, first through a red filter (Wratten No. 25) and then through a blue filter (Wratten No. 47A), the latter exposure being carefully made so as to give just sufficient exposure to the type I emulsion, but insufficient to affect the type II emulsion. In the present instance, the drawing or map was illuminated with white light by means of a 500 candle-power tungsten lamp at two feet away and the sensitive material exposed in a camera, the exposure time being 3 minutes for the red filter and 10 seconds for the blue filter.

The exposed plate was then immersed in the following "surface" developer solution at 70° F.

|                                |       |       |
|--------------------------------|-------|-------|
| N-methyl-p-aminophenol sulfate | grams | 1.1   |
| Sodium sulfite (anhy.)         | do    | 37.5  |
| Hydroquinone                   | do    | 8.5   |
| Sodium carbonate (anhy.)       | do    | 32.5  |
| Potassium bromide              | do    | 1.4   |
| Water to make                  | cc    | 1,000 |

After 30 seconds immersion in this developer solution, the plate was given a uniform exposure for 10 seconds to an ordinary 40-watt electric lamp at 5 feet distance through a blue filter (Wratten 47A). Development was then continued for a total of 4 minutes. The contrasts obtained in the resulting negative and positive images were for all practical purposes the same and only the record of the blue lines was substantially clear in both images. Hence by printing from the finished material, a positive print of only the original blue lines can be made.

The accompanying drawings show a flow-diagram which depicts graphically the process described in the foregoing example. In the first sheet of drawings at B is shown a support coated with first a layer of a red sensitive low blue speed silver chloride emulsion which forms surface latent image on the surfaces of the grains and on top of the first emulsion layer, a layer of a silver bromiodide emulsion which forms latent image mostly inside the silver halide grains, the emulsion having high speed in the blue to blue-green portion of the spectrum and little or no green or red sensitivity. Upon exposure of the two-layer element shown at B to the lighted coloured object shown at A through a red filter, negative latent image is formed on the surface of the silver halide grains in the lower layer as shown at C. Upon then exposing the two-layer element to the coloured object shown at A through a blue filter negative latent image is formed mostly inside the silver halide grains in the upper layer as shown at D. Upon then immersing the two-layer element in a "surface" developer, that part of the upper emulsion layer which does not contain negative latent image is rendered capable of forming surface latent image as shown at E.

Upon exposing the two-layer element to uniform blue light, the upper emulsion layer forms reversed latent image on the surface of the silver halide grains as shown at F (second sheet of drawings). Upon developing the two-layer element in the "surface" developer, the reversed latent image in the upper layer and the negative latent image in the lower layer develops as shown at G. Thus, there is obtained a material in which only the record of the blue portion of the original object is substantially clear. From this material a positive print of only the original blue portion can be made.

It will be observed that although a straightforward photograph taken on any ordinary emulsion layer through a minus blue filter in known manner will selectively record the blue, it will also record black lines whereas the method illustrated in the foregoing example records the blue lines but not the black lines nor any red or green lines, i. e. lines absorbing blue and reflecting red or green. Thus where black lines cross blue lines in the original, there result gaps in the blue lines on the final print obtained as above. The reason that the record of the blue lines is the only clear portion common to both said images is that the negative image (i. e. the red record) is clear only where the red is entirely absent (i. e. where red is not reflected, for instance, where there are blue and black lines) and the positive image (i. e. the blue record) is clear only where blue is present (i. e. where blue is reflected, for instance where there are blue lines, magenta lines and white areas). Where I refer to a part of an image being "clear," I mean only that that part is very much more transparent than the remainder of the image.

Emulsions of type I, i. e. photographic silver salt emulsions which form the latent image mostly inside the silver salt grains have found little or no commercial use heretofore, in fact they have for a long time been considered as practically useless. An example of such type of emulsion is Burton's emulsion given in Wall's "Photographic Emulsions," 1929, pp. 52 to 53. This type of emulsion can be prepared in other known manners, for instance by taking an ordinary gelatino-silver-bromiodide emulsion containing between 0.5 per cent and 5 per cent silver iodide (based on the total silver halide) and coating the emulsion as a layer and then after drying, treating the emulsion with the following bath:

|                      |       |       |
|----------------------|-------|-------|
| Potassium dichromate | grams | 12    |
| Conc. sulfuric acid  | cc    | 12    |
| Water                | cc    | 1,000 |

The time of treatment must be sufficient to inhibit surface latent image formation as can be easily ascertained by exposing (after washing) and then treating with developers of Formulas I and III, given below. Such an emulsion can then be used as it is or may be remelted and coated again as desired.

The emulsions employed in the instant invention are characterized by their behavior in "surface" and "internal" developers. Such developers are given below under Formulas I, II (a), II (b) and III:

#### FORMULA I

##### "Surface" developer

|                                |       |       |
|--------------------------------|-------|-------|
| p-Hydroxyphenylglycine         | grams | 10    |
| Sodium carbonate (crystalline) | do    | 100   |
| Water to                       | do    | 1,000 |

Development time 4 minutes at 20° C.

## FORMULA II (a)

## "Internal" developer

|                                  |       |          |
|----------------------------------|-------|----------|
| Hydroquinone                     | grams | 15       |
| N-methyl-p-aminophenol sulfate   | do    | 15       |
| Sodium sulfite (anhydrous)       | do    | 50       |
| Potassium bromide                | do    | 10       |
| Sodium hydroxide                 | do    | 25       |
| Sodium thiosulfate (crystalline) | do    | 20       |
| Water to                         | cc    | 1,000 10 |

Development time 3 minutes at 20° C.

## FORMULA II (b)

## "Internal" developer

|                                  |       |       |
|----------------------------------|-------|-------|
| Hydroquinone                     | grams | 12    |
| N-methyl-p-aminophenol sulfate   | do    | 3     |
| Sodium sulfite (crystalline)     | do    | 90    |
| Potassium bromide                | do    | 4     |
| Sodium carbonate (crystalline)   | do    | 150   |
| Sodium thiosulfate (crystalline) | do    | 20    |
| Water to                         | cc    | 1,000 |

Development time 4 minutes at 20° C.

## FORMULA III

## Commercial developer

This is the same as Formula II (b), but omitting the sodium thiosulfate.

Formula II (a) is a more energetic developer than Formula II (b) so that it usually gives a higher effective speed and a higher contrast than Formula II (b) but is often not so convenient, since it has a higher tendency to aerial oxidation and to give fog.

While in this specification we have described our invention partly in regard to a theory of internal and surface latent images, the correctness or otherwise of such theory, is not essential to the successful working of the invention, it being only necessary to choose the emulsions according to the tests hereinafter given.

The present invention employs the following types of emulsions:

## TYPE I

These are the emulsions which will develop (after exposure to light) in internal developers of the kind given in at least one of Formulae II (a) and II (b), but will not develop or only slightly develop in Formula III or in Formula I, i. e.; the surface developers.

## (1) Normal range of exposures

As measured according to normal photographic testing technique, when a test layer of the type I emulsion is coated on a transparent support (e. g. glass) and the layer is exposed to a light intensity scale the whole of which is exposed for some fixed time between  $1/100$  and 1 second and is developed in the internal developer II (a), the transmitted density obtained at any point along the  $\log_{10}E$  axis over a range of 3.0 starting from the threshold of the curve ( $D=0.1$  above fog) should be at least 5 times, and preferably at least 10 times the transmitted density obtained when an identical test layer of the emulsion is developed with the surface developer of Formula I or III, the measurements of density being made at the corresponding (i. e. the same) points of the  $\log_{10}E$  axis.

## (2) Small range of exposures

For this purpose the emulsion need not conform to such a rigid requirement, for instance for making a tone correcting mask, but it is sufficient if in the above test the upper limit of 3.1 is substituted by an upper limit of 1.0.

## TYPE II

These are the emulsions which when exposed to a light intensity scale, the whole of which is exposed for some fixed time between  $1/100$  and 1 second, will develop normally in Formulae I and III as well as in Formulae II (a) and II (b). As measured according to normal photographic testing technique, when a test layer of the emulsion is coated on a transparent support (e. g. glass) and the layer is exposed to a light intensity scale the whole of which is exposed for some fixed time between  $1/100$  and 1 second and is developed in the internal developer II (b), the transmitted density obtained at any point along the  $\log_{10}E$  axis of the curve between the range of 0 to 3.0 and preferably between the range of 0 to 2.0 does not exceed the transmitted density obtained when an identical test layer of the emulsion is developed in Formula III, the measurements of density being made at the same points on the  $\log_{10}E$  axis of the curve.

Since Formula III contains sodium sulphite and Formula I is free from sulphite, and sulphite is known to have some solvent action on silver chloride and bromide (although very little on silver iodide), it is apparent that when testing an emulsion to obtain, with a high degree of precision, information on the amount of surface latent image given by such emulsion, it is important to use Formula I. Nevertheless where, as will be apparent hereinafter, in performing the invention a small amount of development of the internal latent image is of no real consequence for practical purposes, it may be advisable to employ Formula III, since this developer is not only less liable to aerial oxidation but gives better density in the image produced by the development of the type II emulsion.

It is to be noted that an "internal" developer is necessarily capable of developing not only a latent image inside grains but also of developing a latent image on the surface of grains (whether such grains contain internal latent image or not) and also of carrying on the development of a surface latent image which has previously been only partly developed.

It is also to be noted that where a "surface" developer is employed to develop a surface latent image, then all grains which are thereby fully developed cannot be subsequently developed at all in an "internal" developer.

This application is a continuation-in-part of my application Serial No. 641,406, filed January 15, 1946.

What I claim as my invention and desire to be secured by Letters Patent of the United States is:

1. The method of selectively producing images in a photographic material comprising, inseparably combined and extending over the same area on a single support, two photographic emulsions, one of said emulsions being a light-sensitive silver salt emulsion (I) a test layer of which is coated upon a transparent glass support upon exposure to a light intensity scale for a fixed time between  $1/100$  and 1 second and development for 3 minutes at 20° C. in the following developer (IIa):

|                                 |       |       |
|---------------------------------|-------|-------|
| Hydroquinone                    | grams | 15    |
| N-methyl-p-aminophenol sulphate | do    | 15    |
| Sodium sulphite, anhydrous      | do    | 10    |
| Potassium bromide               | do    | 10    |
| Sodium hydroxide                | do    | 25    |
| Sodium thiosulphate, crystals   | do    | 20    |
| Water to                        | cc    | 1,000 |

gives a transmitted density at any point along the  $\log_{10}E$  axis, over a range of 1.0 starting from the

threshold of the characteristic curve beginning at a density of 0.1 above fog, at least 5 times the transmitted density obtained when an identical test layer of the emulsion is developed for 4 minutes at 20° C. in the following developer (I):

p-Hydroxyphenylglycine \_\_\_\_\_ grams 10  
Sodium carbonate, crystals \_\_\_\_\_ do 100  
Water to \_\_\_\_\_ cc 1,000

the measurements of density being made at the same points on the  $\log_{10}E$  axis, and the other of said emulsions being a light-sensitive silver salt emulsion (II) a test layer of which coated on a transparent glass support upon exposure to a light intensity scale for a fixed time between  $\frac{1}{100}$  and 1 second and development for 4 minutes at 20° C. in the following developer (IIb):

Hydroquinone \_\_\_\_\_ grams 12  
N-methyl-p-aminophenol sulphate \_\_\_\_\_ do 3  
Sodium sulphite, crystals \_\_\_\_\_ do 90  
Potassium bromide \_\_\_\_\_ do 4  
Sodium carbonate, crystals \_\_\_\_\_ do 150  
Sodium thiosulphate, crystals \_\_\_\_\_ do 20  
Water to \_\_\_\_\_ cc 1,000

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

Hydroquinone \_\_\_\_\_ grams 12  
N-methyl-p-aminophenol sulphate \_\_\_\_\_ do 3  
Sodium sulphite, crystals \_\_\_\_\_ do 90  
Potassium bromide \_\_\_\_\_ do 4  
Sodium carbonate, crystals \_\_\_\_\_ do 150  
Water to \_\_\_\_\_ cc 1,000

the measurements of density being made at the same points on the  $\log_{10}E$  axis of the curve, comprising selectively exposing both emulsions to a lighted object or image to form latent image in both emulsions, treating the photographic material to render the emulsion (I) capable of forming latent image developable by the aforesaid developer (III), then uniformly exposing to light the photographic material to produce latent image in emulsion (I) some of which is developable by the aforesaid developer (III), said uniform exposure to light being insufficient to have any practical effect on said emulsion (II), then developing the photographic material in a developer which develops the latent image developable by said developer (III) and gives no more than a negligible development of the negative latent image formed by the original exposure in emulsion (I) compared with the positive image which is developed in said emulsion (I).

2. The method of selectively producing images in a photographic material comprising, inseparably combined and extending over the same area on a single support, two photographic emulsions, one of said emulsions being a light-sensitive silver salt emulsion (I) a test layer of which coated upon a transparent glass support upon exposure to a light intensity scale for a fixed time between  $\frac{1}{100}$  and 1 second and development for 3 minutes at 20° C. in the following developer (IIa):

Hydroquinone \_\_\_\_\_ grams 15  
N-methyl-p-aminophenol sulphate \_\_\_\_\_ do 15  
Sodium sulphite, anhydrous \_\_\_\_\_ do 10  
Potassium bromide \_\_\_\_\_ do 10  
Sodium hydroxide \_\_\_\_\_ do 25  
Sodium thiosulphate, crystals \_\_\_\_\_ do 20  
Water to \_\_\_\_\_ cc 1,000

gives a transmitted density at any point along the  $\log_{10}E$  axis, over a range of 3.0 starting from the

threshold of the characteristic curve beginning at a density of 0.1 above fog, at least 5 times the transmitted density obtained when an identical test layer of the emulsion is developed for 4 minutes at 20° C. in the following developer (I):

p-Hydroxyphenylglycine \_\_\_\_\_ grams 10  
Sodium carbonate, crystals \_\_\_\_\_ do 100  
Water to \_\_\_\_\_ cc 1,000

the measurements of density being made at the same points on the  $\log_{10}E$  axis, and the other of said emulsions being a light-sensitive silver salt emulsion (II) a test layer of which coated on a transparent glass support upon exposure to a light intensity scale for a fixed time between  $\frac{1}{100}$  and 1 second and development for 4 minutes at 20° C. in the following developer (IIb):

Hydroquinone \_\_\_\_\_ grams 12  
N-methyl-p-aminophenol sulphate \_\_\_\_\_ do 3  
Sodium sulphite, crystals \_\_\_\_\_ do 90  
Potassium bromide \_\_\_\_\_ do 4  
Sodium carbonate, crystals \_\_\_\_\_ do 150  
Sodium thiosulphate, crystals \_\_\_\_\_ do 20  
Water to \_\_\_\_\_ cc 1,000

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III):

Hydroquinone \_\_\_\_\_ grams 12  
N-methyl-p-aminophenol sulphate \_\_\_\_\_ do 3  
Sodium sulphite, crystals \_\_\_\_\_ do 90  
Potassium bromide \_\_\_\_\_ do 4  
Sodium carbonate, crystals \_\_\_\_\_ do 150  
Water to \_\_\_\_\_ cc 1,000

the measurements of density being made at the same points on the  $\log_{10}E$  axis of the curve, comprising selectively exposing both emulsions to a lighted object or image to form latent image in both emulsions, treating the photographic material to render the emulsion (I) capable of forming latent image developable by the aforesaid developer (III), then uniformly exposing to light the photographic material to produce latent image in emulsion (I) some of which is developable by the aforesaid developer (III), said uniform exposure to light being insufficient to have any practical effect on said emulsion (II), then developing the photographic material in a developer which develops the latent image developable by said developer (III) and gives no more than a negligible development of the negative latent image formed by the original exposure in emulsion (I) compared with the positive image which is developed in said emulsion (I).

3. The method of selectively producing images in a photographic material comprising, inseparably combined and extending over the same area on a single support, two photographic emulsions, one of said emulsions being a light-sensitive silver halide emulsion (I) a test layer of which coated upon a transparent glass support upon exposure to a light intensity scale for a fixed time between  $\frac{1}{100}$  and 1 second and development for 3 minutes at 20° C. in the following developer (IIa):

Hydroquinone \_\_\_\_\_ grams 15  
N-methyl-p-aminophenol sulphate \_\_\_\_\_ do 15  
Sodium sulphite, anhydrous \_\_\_\_\_ do 10  
Potassium bromide \_\_\_\_\_ do 10  
Sodium hydroxide \_\_\_\_\_ do 25  
Sodium thiosulphate, crystals \_\_\_\_\_ do 20  
Water to \_\_\_\_\_ cc 1,000

gives a transmitted density at any point along

## 11

the  $\log_{10}E$  axis, over a range of 3.0 starting from the threshold of the characteristic curve beginning at a density of 0.1 above fog, at least 5 times the transmitted density obtained when an identical test layer of the emulsion is developed for 4 minutes at 20° C. in the following developer (I) :

|                            |       |       |
|----------------------------|-------|-------|
| p-Hydroxyphenylglycine     | grams | 10    |
| Sodium carbonate, crystals | do    | 100   |
| Water to                   | cc    | 1,000 |

the measurements of density being made at the same points on the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the following developer (IIb) :

|                                 |       |       |
|---------------------------------|-------|-------|
| Hydroquinone                    | grams | 12    |
| N-methyl-p-aminophenol sulphate | do    | 3     |
| Sodium sulphite, crystals       | do    | 90    |
| Potassium bromide               | do    | 4     |
| Sodium carbonate, crystals      | do    | 150   |
| Sodium thiosulphate, crystals   | do    | 20    |
| Water to                        | cc    | 1,000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III) :

|                                 |       |       |
|---------------------------------|-------|-------|
| Hydroquinone                    | grams | 12    |
| N-methyl-p-aminophenol sulphate | do    | 3     |
| Sodium sulphite, crystals       | do    | 90    |
| Potassium bromide               | do    | 4     |
| Sodium carbonate, crystals      | do    | 150   |
| Water to                        | cc    | 1,000 |

the measurements of density being made at the same points on the  $\log_{10}E$  axis of the curve, comprising selectively exposing both emulsions to a lighted object or image to form latent image in both emulsions, treating the photographic material to render the emulsion (I) capable of forming latent image developable by the aforesaid developer (III), then uniformly exposing to light the photographic material to produce latent image in emulsion (I) some of which is developable by the aforesaid developer (III), said uniform exposure to light being insufficient to have any practical effect on said emulsion (II), then developing the photographic material in a developer which develops the latent image developable by said developer (III) and gives no more than a negligible development of the negative latent image formed by the original exposure in emulsion (I) compared with the positive image which is developed in said emulsion (I).

4. The method of selectively producing images in a photographic material comprising, in separably combined and extending over the same area on a single support, two photographic emulsions, one of said emulsions being a light-sensitive silver halide emulsion (I) a test layer of which coated upon a transparent glass support upon exposure to a light intensity scale for a fixed time between  $\frac{1}{100}$  and 1 second and development for 3 minutes at 20° C. in the following developer (IIa) :

|                                 |       |    |
|---------------------------------|-------|----|
| Hydroquinone                    | grams | 15 |
| N-methyl-p-aminophenol sulphate | do    | 15 |
| Sodium sulphite, anhydrous      | do    | 10 |

## 12

|                               |       |       |
|-------------------------------|-------|-------|
| Potassium bromide             | grams | 10    |
| Sodium hydroxide              | do    | 25    |
| Sodium thiosulphate, crystals | do    | 20    |
| Water to                      | cc    | 1,000 |

gives a transmitted density at any point along the  $\log_{10}E$  axis, over a range of 3.0 starting from the threshold of the characteristic curve beginning at a density of 0.1 above fog, at least 10 times the transmitted density obtained when an identical test layer of the emulsion is developed for 4 minutes at 20° C. in the following developer (I) :

|                            |       |       |
|----------------------------|-------|-------|
| p-Hydroxyphenylglycine     | grams | 10    |
| Sodium carbonate, crystals | do    | 100   |
| Water to                   | cc    | 1,000 |

the measurements of density being made at the same points on the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the following developer (IIb) :

|                                 |       |       |
|---------------------------------|-------|-------|
| Hydroquinone                    | grams | 12    |
| N-methyl-p-aminophenol sulphate | do    | 3     |
| Sodium sulphite, crystals       | do    | 90    |
| Potassium bromide               | do    | 4     |
| Sodium carbonate, crystals      | do    | 150   |
| Sodium thiosulphate, crystals   | do    | 20    |
| Water to                        | cc    | 1,000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the following developer (III) :

|                                 |       |       |
|---------------------------------|-------|-------|
| Hydroquinone                    | grams | 12    |
| N-methyl-p-aminophenol sulphate | do    | 3     |
| Sodium sulphite, crystals       | do    | 90    |
| Potassium bromide               | do    | 4     |
| Sodium carbonate, crystals      | do    | 150   |
| Water to                        | cc    | 1,000 |

the measurements of density being made at the same points on the  $\log_{10}E$  axis of the curve, comprising selectively exposing both emulsions to a lighted object or image to form latent image in both emulsions, treating the photographic material to render the emulsion (I) capable of forming latent image developable by the aforesaid developer (III), then uniformly exposing to light the photographic material to produce latent image in emulsion (I) some of which is developable by the aforesaid developer (III), said uniform exposure to light being insufficient to have any practical effect on said emulsion (II), then developing the photographic material in a developer which develops the latent image developable by said developer (III) and gives no more than a negligible development of the negative latent image formed by the original exposure in emulsion (I) compared with the positive image which is developed in said emulsion (I).

5. The method of selectively producing images in a photographic material comprising, in separably combined and extending over the same area on a single support, two photographic emulsions, one of said emulsions being a light-sensitive silver halide emulsion (I) a test layer of which coated upon a transparent glass support upon exposure to a light intensity scale for a fixed time between  $\frac{1}{100}$  and 1 second and development for 3 minutes at 20° C. in the following developer (IIa) :

|                                 |       |    |
|---------------------------------|-------|----|
| Hydroquinone                    | grams | 15 |
| N-methyl-p-aminophenol sulphate | do    | 15 |
| Sodium sulphite, anhydrous      | do    | 10 |

## 13

$\frac{1}{100}$  and 1 second and development for 4 minutes at 20° C. in the following developer (IIIb):

|                                 |       |       |
|---------------------------------|-------|-------|
| Hydroquinone                    | grams | 12    |
| N-methyl-p-aminophenol sulphate | do    | 3     |
| Sodium sulphite, crystals       | do    | 90    |
| Potassium bromide               | do    | 4     |
| Sodium carbonate, crystals      | do    | 150   |
| Sodium thiosulphate, crystals   | do    | 20    |
| Water to                        | cc    | 1,000 |

gives a transmitted density at any point along the  $\log_{10}E$  axis of the curve between the range of 0 to 2.0 which does not exceed the transmitted density obtained when an identical test layer of the emulsion (II) is developed for 4 minutes at 20° C. in the aforesaid developer (III), the measurements of density being made at the same points along the  $\log_{10}E$  axis, comprising selectively exposing both emulsions to a lighted object or image to form latent image in both emulsions,

|                                 |       |       |
|---------------------------------|-------|-------|
| Hydroquinone                    | grams | 12    |
| N-methyl-p-aminophenol sulphate | do    | 3     |
| Sodium sulphite, crystals       | do    | 90    |
| Potassium bromide               | do    | 4     |
| Sodium carbonate, crystals      | do    | 150   |
| Water to                        | cc    | 1,000 |

the measurements of density being made at the same points along the  $\log_{10}E$  axis, and the other of said emulsions being a light-sensitive silver halide emulsion (II) a test layer of which coated on a transparent glass support upon exposure to a light intensity scale for a fixed time between  $\frac{1}{100}$  and 1 second and development for 4 minutes at 20° C. in the aforesaid developer (IIIb) gives a transmitted density at any point along

## 14

the  $\log_{10}E$  axis of the curve between the range of 0 to 2.0 which does not exceed the transmitted density obtained when an identical test layer of the emulsion (II) is developed for 4 minutes at 20° C. in the aforesaid developer (III), the measurements of density being made at the same points along the  $\log_{10}E$  axis, comprising selectively exposing both emulsions to a lighted object or image to form latent image in both emulsions, 5 treating the photographic material to render the emulsion (I) capable of forming latent image developable by the following developer (I):

|                            |       |       |
|----------------------------|-------|-------|
| p-Hydroxyphenylglycine     | grams | 10    |
| Sodium carbonate, crystals | do    | 100   |
| Water to                   | cc    | 1,000 |

then uniformly exposing to light the photographic material to produce latent image in emulsion (I) some of which is developable by the aforesaid developer (I), said uniform exposure to light being insufficient to have any practical effect on said emulsion (II), then developing the photographic material in a developer which develops the latent image which is developable by the aforesaid developer (I) and gives no more than a negligible development of the negative latent image formed by the original exposure in emulsion (I) compared with the positive image which is developed in said emulsion (I).

6. The process according to claim 5 wherein the two emulsions (I) and (II) are differentially color-sensitized.

GUY WILLIAM WILLIS STEVENS.

No references cited.

**Certificate of Correction**

Patent No. 2,457,005.

December 21, 1948.

**GUY WILLIAM WILLIS STEVENS**

It is hereby certified that errors appear in the printed specification of the above numbered patent requiring correction as follows:

Column 1, line 37, for the word "that" read *and*; column 6, line 74, Formula 1, for "Water to ----- do ---- 1,000" read *Water to ----- cc ---- 1,000*; and that the said Letters Patent should be read with these corrections therein that the same may conform to the record of the case in the Patent Office.

Signed and sealed this 24th day of May, A. D. 1949.

**[SEAL]**

**THOMAS F. MURPHY,**  
*Assistant Commissioner of Patents.*